

## UNITED STATES PATENT OFFICE

2,093,468

## PROCESSING OF TEXTILE YARNS OR THREADS

Abraham Moscowitz, New York, N. Y., assignor  
to L. Sonneborn Sons, Inc., a corporation of  
Delaware

No Drawing. Application October 9, 1936  
Serial No. 104,830

## 18 Claims.

(Cl. 28—1)

This invention relates to new and useful improvements in the processing of textile yarns or threads consisting of natural silk and adapted to be used in the knitting or weaving of textile fabrics.

In the knitting or weaving of textile fabrics with silk yarns or threads the latter are impregnated prior to the knitting or weaving operation with a so called "silk soaking oil". The conventional soaking oils usually comprise in their composition a sulphonated vegetable oil and a straight, that is unsulphonated vegetable oil or fat. The most commonly used sulphonated vegetable oil is olive oil. Among the unsulphonated or straight vegetable oils and fats mostly raw olive oil, neat's-foot oil, cocoanut fat and others of a like nature are used.

The conventional soaking oils, however, present in their application as processing agents for natural silk a series of difficulties, disadvantages and drawbacks which considerably impair their usefulness. The penetrative power of such oils is rather limited and the exhaustion or so called "take-up" of the treating bath is highly unsatisfactory and uneconomical. They furthermore require a comparatively high addition of alkali, and proper operating conditions of the impregnating bath necessitate pH values in excess of 9 and in most instances of at least 10 or higher particularly when the silk, in accordance with the customary practice, is knitted or woven as raw silk or as partly degummed silk, in which case the comparatively high amounts of alkali are essential to soften the silk gum and thus to support the otherwise insufficient penetrative power of the silk soaking agent. The high pH values are not only very detrimental to the fibers and texture of the silk as such but exercise also a decidedly deleterious effect upon the silk gum in the treatment of natural silk which has not been previously degummed or has been partly degummed, such as raw silk, tussah and shappe. In such cases the gum remaining on the silk fibre coagulates due to the high alkalinity and renders the silk thus spotty and subject to uneven dyeing. This coagulation or "stripping" of the silk gum is particularly harmful in the knitting of silk as it causes a sticking in the knitting machine and the frequent breaking of the threads or twists. I have discovered that I can obviate all these defects, disadvantages and deleterious results by using a silk soaking oil which comprises in its composition a "mahogany sulphonate" in conjunction with a sulphonated vegetable oil or fat and a textile treating oil consisting of one or more animal, vegetable or mineral oils or fats.

The mahogany sulphonate which I use is obtained in the manner well-known in the art by subjecting a lubricating oil stock under sulphonating conditions to the action of fuming sul-

phuric acid, usually a 20% SO<sub>3</sub> containing fuming acid, and recovering the so-called "mahogany petroleum sulphonic acids" or shortly mahogany sulphonic acids or their salts from the acid treated oil after the separation of the same from the acid sludge; the sulphonates may be either recovered as such, as for instance by the process described in the Libenthal Patent No. 2,050,345 (August 11, 1936) and subsequently converted into the sulphonates, or, may be recovered directly as mahogany sulphonates in accordance with the ordinary petroleum refining practice by direct neutralization of the acid treated oil followed by suitable extraction. The mahogany sulphonic acids or mahogany sulphonates constitute a material well defined in its character and properties though as yet unknown in its composition. It is assumed to comprise a series of closely related sulphonic acids or sulphonates as the case may be with a varying number of sulfo groups. Inasmuch, however, as the material obtained in the refining of petroleum oils is substantially uniform and well identifiable, I have termed and will refer to the neutralized sulphonic acids for the purpose of brevity simply as "mahogany sulphonate" and wherever I use this term in the specification or claims I mean a neutralized material obtained by the sulphonation of lubricating oil stock as afore-described.

The sulphonated vegetable oil or fat prescribed as the necessary ingredient in my composition may be any one or mixture of the commercially available sulphonated vegetable oils or fats which are obtained by a sulphonation of vegetable oils or fats such as castor oil, olive oil, cocoanut oil or fat, neat's-foot oil, etc., though I preferably use a sulphonated olive oil.

The textile treating oil that I may use in my composition in conjunction with a mahogany sulphonate and a sulphonated vegetable oil or fat may be any unsulphonated oil or fatty substance habitually used in the treatment of textile fibers and materials and may consist of any suitable animal, vegetable or mineral oil or fat, such as olive oil, castor oil, tea seed oil, neat's-foot oil, palm oil, fish oils, liver oils, blubber oils, cocoanut oil or fat, beef tallow, mutton tallow, Texas Pale oil, white oil, etc., or mixtures thereof. Thus, wherever I use the term "textile treating oil" or "textile oil" as appearing in the specification and claims, I mean to include oils as well as fats and fatty or oily substances of the above-described character and nature.

Hitherto the use of mineral oil in compositions of this nature, despite its highly desirable economical and practical aspects, has never been successfully accomplished due to the fact that the conventional compositions containing mineral oil could not be completely and satisfactorily removed from the treated fibers after the knit-

ting or weaving thereof, thus causing considerable trouble in the subsequent finishing and particularly the dyeing operations. I have discovered that no such limitation exists for the use of even relatively high quantities of mineral oil as a component part of the composition in accordance with my invention and I have found it of advantage and use as the preferred combination in my silk soaking oil a textile treating oil comprising a mixture of a mineral oil with a suitable vegetable oil. The mineral oil may be either any straight, that is unsulphonated mineral oil, or a mineral oil blend. For best results I prefer to use a straight mineral oil such as 100 viscosity Texas Pale oil or a white oil, combined with a suitable vegetable oil such as olive oil, tea seed oil, neat's-foot oil, etc.

I have found that my new silk soaking oil is far superior to the conventional compositions, permitting in many instances, to achieve results which it was hitherto impossible to obtain.

The new composition reduces the surface tension of an aqueous treating bath to which it is added to an extremely high degree, thus acting as an excellent wetting agent and effectuating the best possible uniform and even penetration of the materials to be treated. The surprisingly high penetrative power of the agent in conjunction with a more economical and efficient exhaustion of the treating bath is combined with the very advantageous and highly beneficial factor of a low pH (alkalinity) which for successful operating conditions can be adjusted in the treating bath as low as from pH 8 to pH 9 and in some cases as low as pH 7.

As a result of the favorably low pH, the processing with my soaking oil will not deleteriously affect the silk to be treated and its aqueous suspension or a treating bath to which it has been added is absolutely free from the dreaded coagulation effect upon the silk gum which as a rule commences at a pH of 9.5 and proportionately increases with mounting pH values.

The forceful penetrative power of the new soaking oil assures a speedy and efficient, as well as uniform and even soaking of the materials treated.

In addition to the foregoing advantages the new composition imparts to the silk treated therewith a certain amount of hydroscopicity. In many cases this is not only desirable but requisite so as to insure proper and rapid conditioning, which is particularly essential in the knitting of silk. In the customary conditioning operation the necessary moisture content is imparted to the silk by a series of rather cumbersome and time consuming steps which can now be eliminated by the application of my new soaking oil which intrinsically possesses highly hydroscopic properties and is capable of imputing the same to the silk treated therewith to such an extent that proper conditioning can be rapidly achieved by a very simple procedure such as the passing of the treated silk thread over a moist wick.

The highly efficient softening and lubricating qualities of the new agent when applied in a suitable bath to silk in accordance with my invention, far excel those of the conventional compositions and thus render this agent highly beneficial and useful for lubricating and softening purposes.

The amount of mahogany sulphonate and sulphonated vegetable oil present in the composition should be at least sufficient to convert the

normally water immiscible components, that is the textile oil into water miscible form (e. g. emulsion). In order to obtain best results, however, it is of advantage to use in excess of the minimum quantity and amounts of from 10 to 5 50% mahogany sulphonate and from 10 to 20% sulphonated vegetable oil have proven satisfactory in the majority of cases. It is preferable, however, to maintain the proportion of mahogany sulphonate to sulphonated vegetable oil at 10 approximately 1:1. The textile oil may be present in the composition in amounts ranging between 25 and 65% though I prefer to use a proportion of textile oil to total mahogany sulphonate plus sulphonated vegetable oil present 15 of approximately 3:5. Where I use in my preferred formula as the textile treating oil a mixture of a mineral oil with a vegetable oil I may use of from 5 to 25% mineral oil and from 20 to 40% vegetable oil but preferably a proportion of mineral oil to vegetable oil of approximately 2:3. Inasmuch as the commercial mahogany sulphonate contains varying amounts of mineral oil usually up to 35% mineral oil, it is necessary to include this amount of mineral oil 25 in the calculations while making up the formula and to add only so much additional mineral oil as is desired for a particular composition in question without substantially exceeding the afore-30 recited operating limits. Small amounts of a suitable alcohol such as ethyl alcohol or glycol may be added with advantage to further enhance the efficiency of the soaking oil and may range in amounts from 2.5 to 3.5%. For the purpose 35 of aiding the emulsification of the treating bath it is frequently of advantage though not necessary to add to the novel composition some free alkali preferably not in excess of 0.5% such as from 0.7 to 1.2% of a 44% caustic potash solution. In many instances either the mahogany 40 sulphonate or the sulphonated vegetable oil contains already some alkali and should the same be in excess of 0.5% the ratio of alkalinity and organic acidity of the product must be adjusted so that a 5 to 10% emulsion in water will give a 45 pH of not higher than 9 and not less than 7 to 8 and preferably a pH of 8.5. Water is added in all cases to yield 100% and the composition contains as a rule of from 5 to 12% of water. It is, of course, understood and within the purview of 50 my invention to vary the above amounts to suit particular conditions.

The mahogany sulphonate, as such, should be preferably neutral and substantially free from salts. The sulphonated vegetable oil as used in my composition acts as a stabilizing agent for the raw textile oil and increases the action of the mahogany sulphonate; it should preferably possess a combined  $SO_3$  content of about 7 to 8%, a fat content of approximately 60 to 75% and relative freedom from inorganic salts.

The materials which may be impregnated with my new silk soaking agent in the processing of natural silk for knitting or weaving purposes are not limited to any particular silk but extend to all fibers commonly embraced in the term "natural silk", including such materials as raw silk (ecru), culte, souple, tussah, shappe, etc., as well as mixtures of these materials.

In the practical application of my invention silk skeins are first impregnated with the novel silk soaking oil dispersed or emulsified in an aqueous treating bath, and are thereafter further treated to be made into piece goods that 70 75

## Example 3

|                                               | Per cent |
|-----------------------------------------------|----------|
| Mahogany sulphonate (35% mineral oil content) | 24.0     |
| 65% F. M. sulphonated olive oil               | 26.0     |
| 40% neat's-foot oil                           | 34.0     |
| 100 viscosity Texas Pale oil                  | 12.0     |
| Ethyl alcohol                                 | 3.3      |
| 44% caustic potash                            | 0.7      |
| Water                                         | 10       |
|                                               | 100.0    |

## Example 4

|                                               | Per cent |
|-----------------------------------------------|----------|
| Mahogany sulphonate (35% mineral oil content) | 15       |
| 100% F. M. tea seed oil                       | 24.0     |
| 40% neat's-foot oil                           | 15.0     |
| 100 viscosity Texas Pale oil                  | 24.0     |
| Glycol                                        | 24.0     |
| 44% caustic potash                            | 2.9      |
| Water                                         | 1.1      |
|                                               | 9.0      |
|                                               | 100.0    |

## Example 5

|                                       | Per cent |
|---------------------------------------|----------|
| Mahogany sulphonate (35% oil content) | 24.0     |
| 100% F. M. sulphonated olive oil      | 16.0     |
| 40% neat's-foot oil                   | 36.0     |
| 100 viscosity Texas Pale oil          | 12.0     |
| Ethyl alcohol                         | 2.9      |
| 44% caustic potash                    | 1.1      |
| Water                                 | 8.0      |
|                                       | 35       |
|                                       | 100.0    |

The method of application of the compositions recited in Examples 2 to 5 is identically the same as that described in Example 1.

The foregoing description is by way of illustration and not of limitation, and I am not to be limited to any details but only by the appended claims in which I have endeavored to claim broadly all inherent novelty.

I claim:

1. In the manufacture of piece goods containing threads of natural silk the step which comprises impregnating threads of natural silk with a composition containing mahogany sulphonate, sulphonated vegetable oil, textile treating oil and water, the component parts of said composition being proportioned and present in amounts sufficient to adapt the silk threads impregnated therewith to be made into piece goods.

2. In the manufacture of piece goods containing threads of natural silk the step in accordance with claim 1 in which said textile treating oil is composed of mineral oil and vegetable oil.

3. In the manufacture of piece goods containing threads of natural silk the step which comprises impregnating threads of natural silk with a composition containing mahogany sulphonate, sulphonated vegetable oil, textile treating oil, a small amount of alkali and water, the proportion of mahogany sulphonate to sulphonated vegetable oil being substantially 1:1 and the proportion of textile treating oil to total mahogany sulphonate plus sulphonated vegetable oil present being substantially 3:5.

4. In the manufacture of piece goods containing threads of natural silk the step in accordance with claim 3 in which said textile treating oil is composed of mineral oil and vegetable oil substantially in a proportion of 2:3.

## Example 1

The following materials are thoroughly mixed to form the silk soaking oil:

|                             | Per cent |
|-----------------------------|----------|
| Mahogany sulphonate         | 15.0     |
| Sulphonated olive oil       | 16.5     |
| Neat's-foot oil             | 34.0     |
| White oil or Texas Pale oil | 21.0     |
| Alcohol                     | 3.3      |
| 44% caustic potash          | 0.7      |
| Water                       | 9.5      |
|                             | 100.0    |

From 18 to 30 pounds of the above composition are added to approximately 60 to 70 gallons of water at 85° to 95° F. Approximately 135 pounds of raw silk skeins opened and tied in bundles are soaked in this bath for a period of about 12 hours (open bath method) whereafter the excess moisture is removed in a whizzer, a centrifugal arrangement. The skeins are then further treated in the usual manner to be made into piece goods.

## Example 2

|                                | Per cent |
|--------------------------------|----------|
| Mahogany sulphonate            | 14.5     |
| Sulphonated olive oil          | 16.0     |
| Neat's-foot oil                | 36.0     |
| Texas Pale oil (100 viscosity) | 21.5     |
| Glycol                         | 3.3      |
| 44% caustic potash             | 1.1      |
| Water (to yield 100%)          | 8.6      |
|                                | 100.0    |

5. In the manufacture of piece goods containing threads of natural silk the step which comprises impregnating threads of natural silk with an aqueous impregnating bath containing a silk soaking oil substantially composed of from 10 to 50% mahogany sulphonate, from 10 to 20% sulphonated vegetable oil, from 25 to 65% textile treating oil and from 5 to 12% of water, the component parts of said silk soaking oil being proportioned and present in said impregnating bath in amounts sufficient to adapt the silk impregnated therewith to be made into piece goods. 5
- 10 6. In the manufacture of piece goods containing threads of natural silk the step in accordance with claim 5 in which said textile treating oil contains as a component of said silk soaking oil of from 5 to 25% mineral oil and from 20 to 40% vegetable oil. 15
- 15 7. In the manufacture of piece goods containing threads of natural silk the step which comprises impregnating threads of natural silk with an aqueous impregnating bath containing a silk soaking oil substantially composed of from 10 to 50% mahogany sulphonate, from 10 to 20% sulphonated vegetable oil, from 25 to 65% textile treating oil, from 2.5 to 3.5% alcohol, a small amount of alkali not exceeding 0.5% and from 5 to 12% of water, the component parts of said silk soaking oil being proportioned and present in said impregnating bath in amounts sufficient to adapt the silk impregnated therewith to be made into piece goods. 20
- 20 8. In the manufacture of piece goods containing threads of natural silk the step in accordance with claim 7 in which said textile treating oil contains as a component part of said silk soaking oil of from 5 to 25% mineral oil and from 20 to 40% vegetable oil and in which said impregnating bath substantially contains for every 135 pounds of silk from 18 to 30 pounds of said silk soaking oil substantially dispersed in from 60 to 70 gallons of water. 25
- 25 9. In the manufacture of piece goods containing threads of natural silk the step which comprises impregnating threads of natural silk with an aqueous impregnating bath containing a silk soaking oil substantially composed of mahogany sulphonate, sulphonated vegetable oil, textile treating oil and water, while substantially maintaining in said impregnating bath a pH range of from 7 to 9, the component parts of said silk soaking oil being proportioned and present in said impregnating bath in amounts sufficient to adapt the silk impregnated therewith to be made into piece goods. 30
- 30 10. In the manufacture of piece goods containing threads of natural silk the step in accordance with claim 9 in which said textile treating oil is composed of mineral oil and vegetable oil. 35
- 35 11. In the manufacture of piece goods containing threads of natural silk the step which comprises impregnating threads of natural silk with an aqueous impregnating bath containing a silk soaking oil substantially composed of from 10 to 50% mahogany sulphonate, from 10 to 20% sulphonated vegetable oil, from 5 to 12% water and from 25 to 65% of a textile treating oil consisting of from 5 to 25% mineral oil and from 20 to 40% vegetable oil, while substantially maintaining in said impregnating bath a pH range of from 7 to 9, the component parts of said silk 40
- 40 soaking oil being proportioned and present in said impregnating bath in amounts sufficient to adapt the silk impregnated therewith to be made into piece goods. 45
- 45 12. In the manufacture of piece goods containing threads of natural silk the step in accordance with claim 11 in which a pH of 8.5 is substantially maintained in said impregnating bath. 50
- 50 13. In the manufacture of piece goods containing threads of natural silk the step which comprises impregnating threads of natural silk with an aqueous impregnating bath containing a silk soaking oil substantially composed of from 10 to 50% mahogany sulphonate, from 10 to 20% sulphonated vegetable oil, from 5 to 12% water, from 2.5 to 3.5% alcohol, a small amount of alkali not exceeding 0.5% and from 25 to 65% of a textile treating oil consisting of from 5 to 25% mineral oil and from 20 to 40% vegetable oil, while substantially maintaining in said impregnating bath a pH range of from 7 to 9, the component parts of said silk soaking oil being proportioned and present in said impregnating bath in amounts sufficient to adapt the silk impregnated therewith to be made into piece goods. 55
- 55 14. In the manufacture of piece goods containing threads of natural silk the step in accordance with claim 13 in which a pH of 8.5 is substantially maintained in said impregnating bath and in which said impregnating bath substantially contains for every 135 pounds of silk from 18 to 30 pounds of said silk soaking oil substantially dispersed in from 60 to 70 gallons of water. 60
- 60 15. A processed yarn for piece goods manufacture consisting of threads of natural silk impregnated with a silk soaking oil containing mahogany sulphonate, sulphonated vegetable oil, textile treating oil and water, proportioned and in amounts sufficient to impart to said threads a lubrication and hydroscopicity sufficient to adapt the same to be made into piece goods. 65
- 65 16. A processed yarn for piece goods manufacture in accordance with claim 15 in which said silk soaking oil contains a textile treating oil composed of mineral oil and vegetable oil. 70
- 70 17. A processed yarn for piece goods manufacture consisting of threads of natural silk impregnated with a silk soaking oil containing of from 10 to 50% mahogany sulphonate, from 10 to 20% sulphonated vegetable oil, from 5 to 12% water, from 2.5 to 3.5% alcohol, a small amount of alkali not exceeding 0.5% and from 25 to 65% of a textile treating oil consisting of from 5 to 25% mineral oil and from 20 to 40% vegetable oil, in amounts sufficient to impart to said threads a lubrication and hydroscopicity sufficient to adapt the same to be made into piece goods. 75
- 75 18. A processed yarn for piece goods manufacture consisting of threads of natural silk impregnated with a silk soaking oil containing of from 10 to 50% mahogany sulphonate, from 10 to 20% sulphonated vegetable oil, from 5 to 12% water, from 2.5 to 3.5% alcohol, a small amount of alkali not exceeding 0.5% and from 25 to 65% of a textile treating oil consisting of from 5 to 25% mineral oil and from 20 to 40% vegetable oil, in amounts sufficient to impart to said threads a lubrication and hydroscopicity sufficient to adapt the same to be made into piece goods. 80

ABRAHAM MOSCOWITZ.